

June 7, 1927.

1,631,703

E. SOKAL

INTERNAL COMBUSTION ENGINE

Filed Oct. 18, 1926



INVENTOR.  
*Edward Sokal*  
BY  
*Mayer Lewfield & Wallace*  
ATTORNEYS.

Patented June 7, 1927.

1,631,703

# UNITED STATES PATENT OFFICE.

EDWARD SOKAL, OF BROOKLYN, NEW YORK, ASSIGNOR TO AMERICAN KATALITE CORPORATION, OF BROOKLYN, NEW YORK, A CORPORATION OF DELAWARE.

## INTERNAL-COMBUSTION ENGINE.

Application filed October 18, 1926. Serial No. 422,247.

This invention relates to internal combustion engines, to correlated improvements and discoveries whereby and wherewith the operation thereof is enhanced, and more particularly to the prevention of detonation in the combustion chamber thereof.

An object of the invention is directed to the provision in an internal combustion engine of an improved detonation counteractant.

Another object is to provide an improved method of permanently preventing detonation in an internal combustion engine.

A further object is to provide an improved coating composition which may be affixed to the walls of the combustion chamber of an internal combustion engine to prevent detonation therein.

In my co-pending application, Serial No. 42,583, filed July 9, 1925, I have shown that the tendency toward detonation in an internal combustion engine, particularly the pronounced tendency thereto in high compression engines, may be counteracted by fixedly disposing within the combustion chamber of the engine a material capable of undergoing a reversible endothermic, i. e., heat-absorbing, change within the range of temperatures and amid the other conditions existent in the engine during operation, by means of which a cooling effect is exerted upon the gaseous mixture within the chamber with a resultant counteraction of detonation.

While it is well recognized that detonation of the gaseous mixture within a combustion chamber can be counteracted by cooling the mixture, no theory offered in explanation of this phenomenon has been universally accepted. It is my view that detonation, or knocking, in internal combustion engines, is mainly due to a decomposition or breaking down of the unburned fuel, or in other words, to the dissociation of the larger molecules of the fuel under the influence of heat and pressure into a greater number of smaller molecules, whereby there is caused a sudden rise of pressure. This rise of pressure may not be indicative of the true condition within the whole body of the fuel-air mixture, but is rather in the nature of a localized impact. This view is supported by the following considerations: First, the detonating tendency of various fuels is practically a function of their thermal stability, for example, the tendency to

detonate decreases in the following order: kerosene, ordinary gasoline, aromatic gasoline, benzol, alcohol and hydrogen, and the thermal stability increases in the same order. Second, the indicator diagram of detonating engines shows a very rapid rise of pressure which lasts only a very short period of time, is followed by an equally rapid decline, frequently occurs several times at the beginning of the expansion stroke, the peaks becoming smaller each time, and these rises of pressure are of such short duration that the corresponding pressure volume area is too small to represent an appreciable amount of useful work and hence they manifest themselves as destructive impacts. Third, detonation is accompanied by lost power, deposition of carbon and great loss of heat to the water jacket, which loss of power and deposition of carbon may be considered natural results from the decomposition of the fuel, and the loss of heat to the water jacket is probably due to radiation caused by glowing particles of carbon and to the impacts. Fourth, it has been shown that various factors which cause an increase in the rapidity of combustion and make the combustion more complete have a rather pronounced effect in counteracting detonation. This would seem to follow as an indirect result of the fact that the molecules of the fuel cannot simultaneously undergo a reaction of combustion and of decomposition.

In my co-pending application above referred to, I have disclosed as an exemplification of a detonation counteractant suitable for use in accordance with the invention, a material, the melting point of which is such as to render it capable of undergoing a reversible change from solid to liquid state under the conditions of engine operation, and I have particularly suggested the use of lead, antimony and tellurium.

I have now found as a result of continued experimentation that an especially effective detonation counteractant for such use is a non-fugitive, preferably solid, material which is capable under the conditions of engine operation of undergoing a heat-absorbing (endothermic) change at the higher range of temperatures existent within the combustion chamber of the engine in which it is employed so as to be converted into a different non-fugitive, preferably solid, chemical material, which latter material is

capable under the conditions of engine operation of undergoing, at the lower range of temperatures existent within the combustion chamber, a heat-releasing (exothermic) 5 change so as to restore itself for further heat-absorbing action. It will be realized from the above that I use a material which undergoes a reversible chemical change under operating conditions, and that the 10 original substance disposed within the chamber may contain a material appearing on either side of the equation expressing the change, or both. Accordingly, with a view to simplicity of definition, the term "chemically endothermically reactive material", as 15 hereinafter employed, is to be understood to designate either a material falling within the definition of my improved detonation counteractant given above, or a substance 20 which is convertible into such material under the conditions of engine operation. It will be appreciated in this connection that since the invention relates to internal combustion engines, the term "chemically endothermically reactive material" as employed herein- 25 after includes only such substances as will undergo the desired reactions within the range of temperatures and under the other conditions found within the combustion 30 chamber of the engine in which it is employed.

A chemically endothermically reactive material is particularly advantageous for use as a detonation counteractant within the 35 combustion chamber of an internal combustion engine because of the marked heat absorption during the endothermic reaction, with the consequent high cooling effect upon the gaseous mixture. Furthermore, when 40 there is employed a solid material which is converted into another solid material under the conditions contemplated by the invention, a further advantage is to be found in the elimination of any possibility of the 45 loss of the detonation counteractant by the escape of a material which has been converted into a fluid state.

In the practice of the invention a material 50 capable of undergoing a reversible chemical change which is endothermic during the power stroke, when the temperatures within the chamber are the highest and the consequent tendency toward detonation is the greatest, is fixedly disposed within the combustion 55 chamber of an internal combustion engine, preferably in the form of, or as an ingredient of, a coating applied to certain portions of the walls of said chamber. This coating is especially effective when applied 60 to certain of those portions of the chamber walls which are hottest during operation, as, for example, the exposed surface of the piston and/or the exposed surface of the exhaust valves.

65 The accompanying drawing is a partly

sectional view exemplifying a form of the invention. In this exemplification a cylinder block 1, together with a high compression cylinder head 2, provides a combustion chamber 3 into which the contacts 4 of a 70 spark plug 5 extend. A portion of the wall of the combustion chamber is provided by a piston head 6 on the surface of which is a coating 7 containing a relatively permanent chemically endothermically reactive material. Another portion of the wall of this chamber is provided by the surface of an exhaust valve 8 on which there may also be provided a coating 9 which may also contain a relatively permanent chemically endothermically reactive material. 75 80

As an exemplification of a suitable material for use in accordance with the invention, mention may be made of lead carbonate ( $PbCO_3$ ). This material is convertible 85 into litharge ( $PbO$ ) during the power period of engine operation when the range of temperatures within the chamber is the greatest, and the resultant lead oxide is reconvertible into lead carbonate during those intermediate periods of operation when the range of temperatures within the chamber is lower. This reversible change may be represented chemically by the equation 90



wherein the symbols  $+\Delta$  and  $-\Delta$  indicate absorption and release of heat respectively.

Among the other materials which have been found effective for use in accordance with the invention, mention may be made of basic copper carbonate ( $Cu(OH)_2 \cdot CuCO_3$ ), calcium carbonate ( $CaCO_3$ ), sodium carbonate ( $Na_2CO_3$ ) and potassium carbonate ( $K_2CO_3$ ). While the formulæ of particular carbonates of several metals have been given heretofore for the purpose of clearly exemplifying the invention, it will be appreciated that other carbonates of certain of the metals hereinbefore mentioned, may be employed in certain instances. Basic lead carbonate, for example, reacts to form litharge by the equation 100 105 110



within the range of combustion engine temperatures.

It will, of course, be appreciated that in lieu of a carbonate of any particular element there may be employed an oxide thereof which is convertible into the carbonate under the conditions of engine operation; and the term "substance of the carbonate-oxide type" as used hereinafter, is intended to refer either to a carbonate which is endothermically reactive, or to an oxide, a carbonate, a hydroxide, or other material which is convertible into an endothermically reactive carbonate under the conditions contem- 115 120 125 130

plated by the invention. For example, in lieu of a carbonate of lead, litharge or any other oxide of lead which is convertible into an endothermically reactive carbonate of lead under engine operating conditions, may be employed. There may also be used a mixture of litharge and lead carbonate in suitable proportions, as for example, in substantially equal proportions, whereby the 10 advantages inherent in the use of both materials may be utilized.

The litharge possess a somewhat greater initial adhesiveness than the lead carbonate, but the presence of lead carbonate in the exposed surface of the initial coating, although not indispensable, is desirable, because if litharge is used, its change into lead carbonate being an expansion in volume, may have a tendency to loosen its contact with the surface beneath, while in the case of lead carbonate the initial change being accompanied by a diminution of volume, there is hereby a natural provision made for porosity in the coating to take care of any subsequent 20 changes in volume. It is to be noted in this connection that the chemical changes occurring during ordinary operation probably take place only in the exposed surface layer of the detonation counteractant, and also 25 that even on this layer each molecule of the material is probably not converted under ordinary conditions, but that the reaction occurs merely in a proportion of the molecules sufficient to exert the required cooling effect 30 or to restore the material for further heat absorption, as the case may be.

It is to be understood, moreover, that the invention is in no wise limited to the use of any particular material or class of materials, 40 but is directed broadly to any relatively permanent material capable of undergoing, under the conditions of engine operation, a reversible heat-absorbing chemical change; and further that the term "relatively permanent" is intended to apply not only to the 45 improved detonation counteractant, but also to the substance into which it is changed during heat absorption.

In order properly to secure it to the chamber walls, the improved detonation counteractant, in finely divided form, may be admixed with a suitable binder, such as a silicate. For example, an intimate mixture of a finely divided chemically endothermically 50 reactive material with a silicate binder may be applied in the form of a coating on the exposed surface of the piston head, and/or such other portions of the walls as may be desired. The proportions of active substance to the binder may be varied to the requirements of the particular case, and it has been found that satisfactory results are produced when a mixture containing 25% of subdivided litharge, 25% of lead carbonate, 55 and 50% of a silicate is employed, though

these proportions may be varied widely. The application may be accomplished by cleaning the desired surface area, coating such area with the detonation counteractant, and baking or setting. This procedure may be repeated if desired until several coats have been applied. The amount of the improved detonation counteractant to be applied in a particular type of engine may be readily determined by suitable tests indicating the proper surface area to be coated in order to obtain efficient operation.

At the present time the phenomenon of detonation, or knocking, during the operation of internal combustion engines is of 80 much interest because, other conditions being equal, it is more pronounced with engines of high compression ratios. Accordingly this tendency to detonate with a given fuel becomes practically a limiting factor for improvement in the thermal efficiency and power output through an increase in the compression ratio. This is particularly the case with the "constant volume cycle" type of engine which is used almost exclusively 90 in automobiles and in aeroplanes and also to a considerable extent in small marine and stationary engines.

It is true that there are other limiting factors, such as loss in mechanical efficiency, 95 which may offset the gain in thermal efficiency after a certain increase in the compression ratio, but the limitation due to the injurious effects of detonation becomes operative before these other limiting factors 100 exert their influence. Accordingly, it will be apparent that the present invention, because of the marked effectiveness of a chemically endothermically reactive material as a detonation counteractant, will permit the 105 designing of engines having a higher compression ratio than has heretofore been possible.

Among the other advantages arising through the utilization of the detonation 110 counteractant, mention may be made of the following: lack of detonation or knocking, lower fuel consumption, more flexible operation of the engine, decrease in carbon deposition, and an increase in the thermal efficiency, particularly in connection with the use of high compression engines.

It is, of course, to be understood that the invention does not contemplate the use of a material of such a nature that a compound (such, for example, as an oxide of iron) appearing on either side of the equation expressing the reaction occurring within the chamber, has a known cracking effect or other property which would tend to overbalance the effective anti-detonating effect produced by heat absorption during the endothermic reaction.

While the theory herein presented offers a basis for an understanding of the manner 130

in which the detonation counteractant may function, and while it is supported by known facts, it is to be understood, of course, that the operativeness and practicability of the 5 invention is not dependent upon or limited in any way by the correctness of such theory.

Since certain changes may be made in the detonation counteractant above described, and different embodiments of the invention 10 could be made without departing from the scope thereof, it is intended that all matter contained in the above description shall be interpreted as illustrative and not in a limiting sense.

15 It is also to be understood that the following claims are intended to cover all of the generic and specific features of the invention herein described, and all statements of the scope of the invention which, as a 20 matter of language, might be said to fall therebetween.

Having described my invention, what I claim as new and desire to secure by Letters Patent, is:

25 1. In an internal combustion engine, the combination with a combustion chamber, of a relatively permanent detonation counteractant fixedly disposed within said chamber, and consisting of a material which is 30 chemically endothermically reactive under engine operating conditions.

2. In an internal combustion engine, the combination with a combustion chamber, of a coating disposed on certain of the walls 35 of said chamber, said coating containing a relatively permanent material which is chemically endothermically reactive under engine operating conditions.

3. In an internal combustion engine, the 40 combination with a combustion chamber, of a coating disposed on certain of those portions of the walls of said chamber which are hottest under operating conditions, said coating containing a solid material capable 45 of undergoing, under operating conditions, a reversible endothermic chemical change into other solid material.

4. In an internal combustion engine, a 50 combustion chamber arranged for the reception of a gaseous mixture and fitted with a piston presenting an exposed surface to the gases in said chamber, said surface comprising a coating containing a material which is chemically endothermically reactive under 55 engine operating conditions.

5. In an internal combustion engine, the combination with a combustion chamber, and of a metallic salt which is chemically endothermically reactive under engine operating 60 conditions fixedly disposed within said chamber.

6. In an internal combustion engine, the combination with a combustion chamber, of an endothermically chemically reactive substance 65 of the carbonate-oxide type fixedly

disposed upon certain of the walls of said chamber.

7. In an internal combustion engine, a combustion chamber arranged for the reception of a gaseous mixture and fitted with 70 a piston presenting an exposed surface to the gas in said chamber, said surface comprising a coating containing a carbonate capable of undergoing a reversible change into an oxide under engine operating conditions. 75

8. In an internal combustion engine, the combination with a combustion chamber, of a coating formed on certain of those portions of the walls of said chamber which are hottest during engine operation, said coating 80 containing an endothermically reactive lead compound.

9. In an internal combustion engine, the combination with a combustion chamber, of a detonation counteractant fixedly disposed 85 within said chamber, said detonation counteractant comprising a carbonate of lead.

10. In an internal combustion engine, the combination with a combustion chamber, of a coating formed on certain of those portions 90 of the walls of said chamber which are hottest during operation, said coating comprising normal lead carbonate.

11. In an internal combustion engine, the combination with a combustion chamber, of a detonation counteractant fixedly disposed 95 within said chamber, said detonation counteractant comprising litharge.

12. In an internal combustion engine, the combination with a combustion chamber, of 100 a coating formed on certain of the walls of said chamber, said coating containing a carbonate of lead and litharge.

13. As an article of manufacture, a piston head arranged for use within an internal 105 combustion engine, the pressure surface thereof having formed thereon a coating containing a chemically endothermically reactive lead compound of the carbonate-oxide type. 110

14. In an internal combustion engine, the combination with a combustion chamber, of an endothermically chemically reactive lead compound of the carbonate-oxide type fixedly disposed within said chamber. 115

15. In an internal combustion engine, the combination with a combustion chamber, of a coating formed on certain of the walls of said chamber, said coating containing a relatively permanent material which is chemically endothermically reactive under engine operating conditions, and a binder. 120

16. In an internal combustion engine, the combination with a combustion chamber, of a relatively permanent material which is chemically endothermically reactive under engine operating conditions, in finely divided form, intimately admixed with a silicate binder. 125

17. In an internal combustion engine, the 130

combination with a combustion chamber, of a coating formed on certain portions of the walls of said chamber, said coating containing a carbonate of lead and a silicate.

5 18. A method of effecting improvement in the operation of an internal combustion engine, which comprises permanently exposing within the combustion chamber thereof a material which is chemically endothermically reactive under engine operating conditions.

10 19. A method of counteracting detonation of the successive fuel charges in the combustion chamber of an internal combustion engine, which comprises permanently

exposing to such charges a solid material capable of undergoing, under engine operating conditions, a reversible endothermic chemical change into other solid material.

15 20. A method of effecting improvement in the operation of an internal combustion engine, which comprises forming on certain of those portions of the wall of the combustion chamber of the engine which are the hottest during operation, a coating containing a relatively permanent metallic carbonate which is chemically endothermically reactive under engine operating conditions.

25 In testimony whereof I affix my signature.

EDWARD SOKAL.

combination with a combustion chamber, of a coating formed on certain portions of the walls of said chamber, said coating containing a carbonate of lead and a silicate.

5 18. A method of effecting improvement in the operation of an internal combustion engine, which comprises permanently exposing within the combustion chamber thereof a material which is chemically endothermically reactive under engine operating conditions.

10 19. A method of counteracting detonation of the successive fuel charges in the combustion chamber of an internal combustion engine, which comprises permanently

exposing to such charges a solid material capable of undergoing, under engine operating conditions, a reversible endothermic chemical change into other solid material.

20 20. A method of effecting improvement in the operation of an internal combustion engine, which comprises forming on certain of those portions of the wall of the combustion chamber of the engine which are the hottest during operation, a coating containing a relatively permanent metallic carbonate which is chemically endothermically reactive under engine operating conditions.

25 In testimony whereof I affix my signature.

EDWARD SOKAL.

**Certificate of Correction.**

Patent No. 1,631,703.

EDWARD SOKAL.

Granted June 7, 1927, to

It is hereby certified that error appears in the printed specification of the above-numbered patent requiring correction as follows: Page 1, line 1, for the misspelled word "intenal" read *internal*, and line 49, after the word "true" insert the word *pressure*; page 3, line 81, for the misspelled word "condtions; read *conditions*; and that the said Letters Patent should be read with these corrections therein that the same may conform to the record of the case in the Patent Office.

Signed and sealed this 19th day of July, A. D. 1927.

[SEAL.]

M. J. MOORE,  
*Acting Commissioner of Patents.*

**Certificate of Correction.**

**Patent No. 1,631,703.**

**Granted June 7, 1927, to**

**EDWARD SOKAL.**

It is hereby certified that error appears in the printed specification of the above-numbered patent requiring correction as follows: Page 1, line 1, for the misspelled word "intenal" read *internal*, and line 49, after the word "true" insert the word *pressure*; page 3, line 81, for the misspelled word "condtions" read *conditions*; and that the said Letters Patent should be read with these corrections therein that the same may conform to the record of the case in the Patent Office.

Signed and sealed this 19th day of July, A. D. 1927.

[**SEAL.**]

**M. J. MOORE,**  
*Acting Commissioner of Patents.*